

Aug. 18, 1942.

H. L. MEAD ET AL

**2,293,033**

## APPARATUS AND PROCESS FOR DESLIMING FLOTATION FEED

Filed April 5, 1940

2 Sheets-Sheet 1



INVENTORS  
HARRY L. MEAD,  
ERNEST J. MAUST,  
BY Robert Ames Norton  
ATTORNEY.

Aug. 18, 1942.

H. L. MEAD ET AL

2,293,033

APPARATUS AND PROCESS FOR DESLIMING FLOTATION FEED

Filed April 5, 1940

2 Sheets-Sheet 2

Fig. 2.



INVENTORS  
HARRY L. MEAD,  
ERNEST J. MAUST  
BY  
Robert Ames Morton  
ATTORNEY.

## UNITED STATES PATENT OFFICE

2,293,033

APPARATUS AND PROCESS FOR DESLIMING  
FLOTATION FEEDSHarry L. Mead and Ernest J. Maust, Brewster,  
Fla., assignors to American Cyanamid Company,  
New York, N. Y., a corporation of Maine

Application April 5, 1940, Serial No. 327,948

6 Claims. (Cl. 209—454)

This invention relates to the desliming of flotation feed in the ore dressing art and more particularly it relates to an improved apparatus of the hindered settling type for desliming the finest fraction of flotation feed.

Recent improvements in the flotation art have required that flotation feeds be very thoroughly deslimed, that is to say, more completely than the desliming produced in the use of free settling tanks. This is particularly true in connection with the flotation of silica from phosphate rock using the so-called cationic flotation reagents as even very small quantities of slime have a deleterious effect on the promoter action of the reagents.

In our copending application Serial No. 320,121 filed February 21, 1940, we have described an improved process for the simultaneous sizing and desliming of phosphate ore flotation feed in a hindered settling classifier, which is a much more efficient method than the ordinarily employed desliming operations, the process, however, deals only with the desliming of the larger particle fractions of the phosphate material and does not result in slime removal from the very fine fraction of phosphate material to which the present invention relates.

The ordinary methods of desliming very fine flotation feed in the past have not been found to be entirely satisfactory. The prior methods of desliming very fine ore material usually consists of passing the material into a series of large settling tanks with the addition of large volumes of fresh water to each of the series of settling tanks. Adequate settling area in this case must be provided in each tank to settle all of the plus 250 mesh material each time that it enters a tank. As some slime always tends to settle with true particle size material, the amount of slime settling in each tank of a series is a decreasing amount, but is never entirely removed as mathematically this is impossible. Hence, in previous methods it was not economically practical to obtain the high degree of desliming that is attained in the hydraulic hindered settling deslimer of this invention. The settling tanks of the prior methods might be cylindrical tanks with flat bottoms, conical tanks, or rectangular tanks with bowl attachments wherein the settled material was raked out of the bath.

In accordance with the present invention a process is provided in which very fine fractions of flotation feed can be thoroughly deslimed. An improved apparatus of the hindered settling type is provided in which the entire desliming opera-

tion is conducted in one tank where a small amount of water and a small area does work equivalent to that accomplished by a series of large settling tanks employing much larger quantities of water. This improved apparatus is useful for desliming very fine flotation feed of any ore material but it is particularly useful in the non-metallic field, especially the finest fraction of phosphate flotation feed ranging from —48 mesh down to 325 mesh.

In carrying out our invention use is made of the density of a teetering mass of fine flotation feed to keep the light slime from entering the denser body of material in suspension. A density in excess of that of water is induced in the pockets of the hindered settling deslimer due to the particles being held in teeter by means of the hydraulic water passing through the constriction plate in the bottom of the compartment. Hence, in addition to the tendency for a rising column of water to carry off slime, the density of the material in suspension also tends to aid in slime removal. In our improved hindered settling deslimer water is added at such a rate that only about 6 gallons per minute per square foot of overflow area is used. In the ordinary hindered settling classifier water in excess of this amount must be used to keep the particles in suspension and thus fine flotation feed is overflowed. This water limitation at a point of not over about 6 gallons per minute per square foot of overflow area is made possible and teeter still maintained by flaring the hydraulic chamber at a point above the teeter column.

It is an advantage of the present invention that the finest fraction of phosphate flotation feed which cannot be deslimed in the ordinary hindered settling classifier (—48 mesh down to 325 mesh) is readily deslimed using our improved apparatus. A very thoroughly deslimed product is produced, which deslimed feed when subjected to froth flotation concentration by either the silica flotation process or the fatty acid phosphate flotation process results in a higher grade product and permits more efficient operation.

The present invention has many advantages over the prior desliming processes such as those using a series of settling tanks or cones, drag classifiers and the like. Some of these outstanding advantages are low first cost of equipment, small floor space, and economy of about 60% to 70% in the use of water over the free settling desliming. When compared to a desliming process using a series of these cones it was found

that only  $\frac{1}{3}$  as much water was needed in our improved hindered settling deslimer and at the same time the initial cost was only about  $\frac{1}{5}$  as much to produce a better deslimed product.

The invention will be more readily understood by referring to the following drawings of our improved hindered settling deslimer apparatus in which:

Fig. 1 is a longitudinal sectional view;

Fig. 2 is a top plan view; and

Fig. 3 is a transverse sectional view taken along the lines 3—3 of Figs. 1 and 2 and looking in the direction of the arrows.

The deslimer comprises a tank 1 having the flaring sides 2. The lower half of the tank is divided into a plurality of pockets or compartments as illustrated. These pockets are numbered from 7 to 13 inclusive. A hydraulic water compartment 3 is located beneath the pockets and separated therefrom by the perforated constriction plate 4 through which hydraulic water may be flowed. Any number of pockets may be used, the number being optional and limited only to a practical size over which water may be uniformly distributed through the holes of the constriction plate in the hydraulic water compartment 3. Hydraulic water inlets 22 are shown leading into the various portions of the hydraulic water compartments 3 in such a manner that varying amounts of water and at different velocities may be forced through the constriction plate 4 into each of the pockets 7 to 13 inclusive. A baffle plate 14 divides each of the pockets from the adjoining pockets from 7 to 12 inclusive. All of the pockets except 13 are connected through a suitable opening or slot 15 in the baffles 14. While the slot 15 is shown extending only part way up the baffles 14, it may, if desired, be extended to the top. A standpipe 17 is shown positioned in the pocket 12, in such a manner that changes of specific gravity in this compartment cause water to rise in the pipe actuating a diaphragm 20 operatively connected to the top of the standpipe. This diaphragm may be of the ordinary flexible rubber type but is preferably a bellows diaphragm. When the diaphragm is forced upwardly by water pressure the plumb bob valve 18 which is seated in the discharge opening 19 in the bottom of pocket 13 is raised a sufficient height to permit the deslimed feed to pass out through the opening 19. Each of the pockets 7 to 13 inclusive may for convenience have observation windows 23 which will permit the operator to view the passage of the feed through these compartments. A feed opening 21 is so arranged in conjunction with the baffle 16 that when feed is introduced it passes directly into the compartment 7. An overflow area at the top of the flared portion of tank 2 is provided by means of the weir 5 by which water and slime are overflowed into the overflow launder 6. The weir 24 prevents overflow at the most distant portion of the tank from the feed entrance.

In operation a very fine flotation feed, as for example in the case of phosphate rock ranging in particle size from —48 to 325 mesh, is fed into the feed opening 21 and thence into the compartment 7, whereupon the rising currents of hydraulic water passing through the construction plate 4 carry the finer slime particles into the flared portion of the tank. Here the upward velocity of the water decreases due to the increased area. The velocity is, however, sufficient to carry the slimy particles over the weir 5. The velocity of the water in the flared portion 75

of the tank is not sufficient, however, to support the ore particles and they fall back into the pockets. The feed passes from the pocket 7 into the pocket 8 by means of the slot 15 and is here subjected to hydraulic water at a velocity different from that in pocket 7. This process is repeated as the feed passes from pocket to pocket, additional quantities of slime being removed in each pocket until the thoroughly deslimed feed collects in the last pocket 13, from which it is subsequently discharged by operation of the diaphragm actuated through the changes of specific gravity in pocket 12 to open the plumb bob valve seated in the feed discharge opening 19. There is no opening in the baffle 14 separating pocket 12 from pocket 13 and the velocity of the hydraulic water in 13 is just enough less than that of pocket 12 so that the feed passing over the top of baffle 14 into pocket 13 will settle or collect at the bottom.

We have found that a very fine fraction of phosphate flotation feed can be very thoroughly deslimed in accordance with the above operation, by which even the 250 mesh material may be retained using an apparatus in which approximately 2000 gallons per minute for 50 long tons per hour of feed were being processed. Among the important features which appear to be in a general measure responsible for the improved results of this apparatus are the flared sides of the tank which increase the area and reduce the velocity of the uprising currents of water so that the slimes are carried over the top and the ore materials fall back and can be collected.

By restricting the overflow at a point where the material is to be removed, we provide a positive flow of a small amount of remaining slime in a direction opposite to that of the passage of feed. This is an important part of the invention. Another important part of this invention is the restricting of the flow rate of water in the cell in which the material is discharged to a point low enough to settle all of the plus 250 mesh flotation feed. As water is added in excess of this amount in the other cells, limiting the velocity of upward flow to a point below 6 gallons per minute per square foot of overflow area at the overflow point, the finest of the flotation feed could not settle into the bottom of these pockets to be discharged. Hence, in the pocket through which the material is discharged the velocity of the rising current of water is maintained at a point below 6 gallons per minute per square foot of area. As the fine material is not agitated sufficiently at this low flow rate to actuate a diaphragm discharge mechanism, this mechanism is operated from the super-elevation water in the adjoining pocket to discharge the deslimed feed in the discharge compartment.

In a preferred embodiment of our apparatus a diaphragm actuated device working through super-elevation of the material in teeter in a pocket of the machine to discharge the material, from an adjoining pocket is employed. The deslimed feed might also be discharged by means of a hand operated valve, a centrifugal pump or a simple spigot, without violating the basic features of the invention. There are many advantages however, which result from the use of the teeter column actuated diaphragm pump, among which are: it is automatic in operation and does not require the attention of an operator, it is easily adjusted for any variance in the

type of feed, amount of feed or other operating conditions.

In utilizing our improved apparatus no sizing is attempted unless we differentiate between colloidal slime and true particle size of about 250 mesh. The rising velocity of the hydraulic water is regulated in such a manner that it is sufficient to float away the colloidal slimes while at the same time it is approximately equal to or less than the free settling rate of 250 mesh sand. When the velocity of the rising water is thus regulated the 260 mesh sand and, of course, the material larger than 250 mesh readily separates out and is completely free from the colloidal slimes.

We claim:

1. A method of desliming without classifying slimy ore feed containing fine particle sizes which comprises introducing the feed into a rising column of water the velocity of said rising column being such as to cause the coarsest particles of the feed to remain in suspension, subjecting said stream of water to deceleration to a velocity at which the finest ore particles settle but slime rises, overflowing a portion of the water at said velocity to remove slime, causing said deslimed materials to pass into a zone of rising water the velocity of which is such that the particles just settle in a discharge zone and discharging the settled ore particles from said discharge zone at a rate determined by sensing means located in a zone preceding the discharge zone.

2. A method of desliming without classifying slimy phosphate ore feed containing very fine particle sizes, which comprises introducing the feed into a rising column of water the velocity of said rising column being such to cause the coarsest particles of the feed to remain in suspension, subjecting said stream of water to deceleration to a velocity at which the finest ore particles settle but slime rises, overflowing a portion of the water at said velocity to remove slime, causing said deslimed material to pass into a zone of rising water the velocity of which is such that the finest ore particles just settle in a discharge zone and discharging the settled ore particles from said discharge zone at a rate determined by sensing means located in a zone preceding the discharge zone.

3. A method of desliming without classifying slimy phosphate ore feed containing very fine particle sizes, ranging from -48 to +325 mesh which comprises introducing the feed into a rising column of water the velocity of said rising column being such to cause the coarsest particles of the feed to remain in suspension, subjecting said stream of water to deceleration to a velocity at which the finest ore particles settle but slime rises, overflowing a portion of the water at said velocity to remove slime, causing said deslimed material to pass into a zone of rising water the velocity of which is such that the finest ore, 250 mesh, particles just settle in a discharge zone and discharging the settled ore particles from said discharge zone at a rate determined by sensing means located in a zone preceding the discharge zone.

4. A hindered settling deslimer comprising a

tank the upper portion of which has flared sides and an overflow area for slimes, a series of pockets located in the lower portion of the tank, means for introducing ore material into one of the pockets, means for discharging the coarser ore material in a pocket located at the opposite end of the series from the one into which the feed is introduced, means for introducing water upwardly into each of the pockets at a variable velocity, means for restricting overflow above the pocket from which the deslimed feed is discharged which causes the excess water to flow in a direction opposite to that of the passage of feed water in order to overflow from the tank, said pockets in the series communicating with one another through restricted openings in the sides thereof with the exception that there is no communicating opening in the wall of the discharge pocket.

5. A hindered settling deslimer comprising a tank the upper portion of which has flared sides and an overflow area for slimes, a series of pockets located in the lower portion of the tank and having perforated bottoms, means for introducing ore material into one of the pockets, means for discharging the coarser ore material in a pocket located at the opposite end of the series from the one into which the feed is introduced, means for introducing water through the aforesaid perforated bottoms into each of the pockets at a variable velocity, means for restricting overflow above the pocket from which the deslimed feed is discharged which causes the excess water to flow in a direction opposite to that of the passage of feed water in order to overflow from the tank, said pockets in the series communicating with one another through restricted openings in the sides thereof with the exception that there is no communicating opening in the wall of the discharge pocket and the preceding pocket.

6. A hindered settling deslimer comprising a tank the upper portion of which has flared sides and an overflow area for slimes, a series of pockets located in the lower portion of the tank and having perforated bottoms, means for introducing ore material into one of the pockets, means for discharging the coarser ore material which comprises a diaphragm mechanism actuated by density changes in one pocket to operate a feed discharge opening in the bottom of another pocket located at the opposite end of the series from the one into which the feed is introduced, means for introducing water through the aforesaid perforated bottoms into each of the pockets at a variable velocity, means for restricting overflow above the pocket from which the deslimed feed is discharged which causes the excess water to flow in a direction opposite to that of the passage of feed water in order to overflow from the tank, said pockets in the series communicating with one another through restricted openings in the sides thereof with the exception that there is no communicating opening in the wall of the discharge pocket and the preceding pocket.

HARRY L. MEAD.  
ERNEST J. MAUST.